

Aug. 5, 1958

W. H. KELLER ET AL

2,846,303

METHOD OF PRODUCING TITANIUM

Filed Aug. 11, 1953

2 Sheets-Sheet 1



FIG. 1

INVENTORS  
Wayne H. Keller  
Irwin S. Zonis  
BY

Oliver W. Horrey

ATTORNEY

Aug. 5, 1958

W. H. KELLER ET AL

2,846,303

METHOD OF PRODUCING TITANIUM

Filed Aug. 11, 1953

2 Sheets-Sheet 2



INVENTORS

Wayne H. Keller  
Irwin S. Zonis

Oliver W. Hayes

ATTORNEY

1

2,846,303

## METHOD OF PRODUCING TITANIUM

Wayne H. Keller, Waban, and Irwin S. Zonis, Belmont, Mass., assignors to National Research Corporation, Cambridge, Mass., a corporation of Massachusetts

Application August 11, 1953, Serial No. 373,512

11 Claims. (Cl. 75—84.5)

This invention relates to the production of metals and more particularly to the production of titanium.

A principal object of the present invention is to provide an improved process for the manufacture of titanium and alloys thereof.

Another object of the invention is to provide a process of the above type which produces stable crystals of titanium.

Still another object of the invention is to provide a process of the above type which gives crystals of titanium of sufficiently large size so that aqueous leaching can be employed to separate the product titanium from the by-product salt without contaminating the product titanium.

Still another object of the invention is to provide an improved process for making low-cost titanium having a purity comparable to titanium produced by the iodide process.

Other objects of the invention will in part be obvious and will in part appear hereinafter.

The invention accordingly comprises the process involving the several steps and the relation and the order of one or more of such steps with respect to each of the others which are exemplified in the following detailed disclosure, and the scope of the application of which will be indicated in the claims.

For a fuller understanding of the nature and objects of the invention, reference should be had to the following detailed description taken in connection with the accompanying drawings wherein:

Fig. 1 is a flow sheet illustrating one preferred embodiment of the invention; and

Fig. 2 is a graph illustrating the gradual reduction of valence employed in the specific examples.

The production of titanium metal has recently been the object of an enormous amount of research work by leading industrial concerns throughout the United States and Europe. Many methods have been proposed for the production of titanium, a number of these methods involving the metallothermic reduction of titanium halides. In particular, the magnesium reduction of titanium tetrachloride has begun to assume considerable commercial importance. Most of the prior art processes which employ the rather low-temperature reduction of titanium by the use a liquid metal reducing agent, such as magnesium, have resulted in the production of titanium in a spongy form containing large quantities of entrapped magnesium, magnesium chloride, and lower chlorides of titanium. So far as is known, the product from such a reaction (often referred to as the Kroll process) is extremely difficult to purify and involves hand drilling of the reactor pots with subsequent vacuum leaching of the product titanium.

Other processes (such as the Degussa process practiced in Germany) have resulted in the production of fine titanium powder of a highly pyrophoric nature. This product is equally difficult to separate from the by-product sodium chloride.

These prior art processes, while involving relatively simple metallothermic reduction steps, necessitate enor-

2

mously expensive purification procedures so that the resultant product titanium must be sold at a high price. Additionally, even the drastic precautions taken during purification invariably result in a product which is not as pure as that produced by the much more expensive iodide process.

In the present invention advantage is taken of the well-known ability of the alkali and alkaline earth metals to reduce titanium tetrachloride, for example, to titanium metal. This reaction proceeds rapidly at relatively low temperatures (i. e., temperatures on the order of the melting point of the by-product halide). However, in the present invention the reaction conditions are so adjusted that the product titanium consists of large crystals of titanium which can be removed from the reactor as a slurry of crystalline titanium in the molten salt. These crystals have a size sufficiently large as to permit simple leaching with water (containing a small percentage of acid) to dissolve the by-product halide. The size of the individual crystals is such that the surface-to-volume ratio is relatively low, thereby preventing contamination of the product due to the presence of surface oxide. The nature of the product is also such that its surface activity appears to be very low. Additionally, it is preferred that essentially no lower chlorides of titanium exist in the final product removed from the reactor. Accordingly, the nature of the product and the use of the slightly acid water leach substantially prevent the possibility of appreciable oxidation of the titanium or hydrolysis of any lower titanium halides (with the consequent formation of non-volatile oxides of titanium). Additionally, the product is in such form that, by simple filtration or decantation, the great bulk of the by-product salt can be separated from the titanium crystals so that the amount of leaching is kept to a minimum. This is particularly advantageous in those cases where the recycling of an anhydrous salt to electrolytic alkali metal or alkaline earth metal cells is an integral part of the over-all operation.

In a preferred method of practicing the present invention, there is provided, in an air-free reduction zone, a mixture of a molten salt and at least one lower chloride of titanium, this mixture being essentially free of titanium fines. The lower chloride content of this mixture is then gradually reduced from an average titanium valence of 3 or less to a valence of zero. For convenience, this reduction of the lower chlorides is often hereinafter referred to as the "final reduction" step. The mixture of lower chlorides provided in the final reduction zone may be formed, in situ, within the final reduction zone by feeding, for example, sodium and titanium tetrachloride into this final reduction zone, the molar ratio of the reactant feed being adjusted so that the titanium tetrachloride is reduced only to a lower chloride or a mixture of lower chlorides. The mixture initially formed in the final reduction zone may comprise, for example, sodium chloride, titanium trichloride, titanium dichloride, and perhaps a small quantity of titanium metal.

In understanding the invention it is convenient to consider the average valence state of the total titanium content (free titanium and titanium chlorides) in the final reduction zone. The initial valence state in the final reduction zone may be as high as 3 or may be as low as 2 or lower. From the standpoint of commercial operation, the preferred initial valence state will depend upon a number of factors. If the titanium chloride charged to the final reduction zone is to be formed by the reduction of titanium tetrachloride with a metallic reducing agent, such as sodium or the like, it is desirable to carry the initial reduction to an average valence state of 2. This initial reduction may be very rapid, if desired, and can take place in a separate reactor feeding a num-

ber of final reduction zones. As far as is known, about the only limitation on the speed of the formation of the mixture of lower halides (so long as the average valence remains as high as 2) is the problem of removal of heat due to the highly exothermic nature of the metallothermic reduction reaction. It is extremely important, however, that the initial production of this mixture be carried out so that formation of titanium fines be prevented. Thus, even though the average titanium valence is as high as 2 or above, the mixture can contain a considerable quantity of titanium fines if the mixture is produced under conditions where localized unbalance in stoichiometry occurs. Accordingly, it is of the utmost importance that the formation of the initial mixture be achieved under the most nearly uniform concentrations of reducing agent and reducible titanium compound. By "titanium fines" is meant titanium particles having a size less than about 200 mesh.

Once the initial charge has been fed to the final reduction zone, the growth of titanium crystals in the final reduction zone is accomplished by the gradual reduction of the average titanium valence to zero. From the standpoint of simplicity of the apparatus, it is preferred that, during the final reduction period, only the reducing agent be fed. It is also highly desirable that the reduction of the average titanium valence be uniformly slow throughout the reaction mass. Thus, with a large reactor, the reducing agent should be uniformly dispersed throughout the reaction mass. One method of achieving this uniform distribution of the reducing agent (e. g., sodium) is to feed the sodium to the top of the salt bath and permit the sodium to diffuse through the bath by dissolving in the salt bath.

It appears desirable to have the final reduction period continue on the order of one hour and preferably in excess of two hours. This final reduction period may be as long as 3 to 5 hours, although not much is gained by having the final reduction period longer than about 5 hours. It appears that the titanium crystal growth takes place in a mixture containing titanium at an average valence state of less than 3 and that maximum growth apparently takes place as the valence state decreases from 2 to zero at a very slow rate.

This titanium crystal growth requires a definite time period, the lower limit of which seems to be on the order of an hour or so, and the upper limit of which is dictated only by economic considerations. It also requires the presence of lower chlorides of titanium (particularly the dichloride), and that reduction of some of the lower chlorides must be taking place during the growth period. This is true even though the average valence state may remain constant. For example, crystal growth can be obtained at a constant average titanium valence state of 1 if a reducing agent and titanium tetrachloride are fed at a constant slow rate to the final reduction zone containing a fused salt and a mixture of titanium and titanium chlorides having an average valence state of 1 (see Example II, infra). On the other hand, a similar mixture of salt, titanium, and titanium chlorides, having an average valence state of 1, when held for a comparable length of time at a comparable temperature produces much less crystal growth if a reducing agent is not present. Thus, as mentioned previously, the growth period is preferably one in which reduction of lower chlorides of titanium takes place. There may additionally be present a number of back reactions, such as the reaction between titanium trichloride and titanium metal, or the reaction between titanium dichloride and titanium tetrachloride. There may also be present some disproportionation of titanium dichloride and trichloride. It is also quite conceivable (although its existence has not been established) that titanium monochloride may exist in the system, in at least a transitory form, and may contribute in a significant manner to the crystal growth reaction.

In one preferred method of practicing the invention, 75

titanium tetrachloride and sodium, for example, are fed to a final reduction zone at a relatively high rate. This final reduction zone may have an initial charge of sodium chloride which is maintained at a temperature above its melting point. The relative feed rates of the titanium tetrachloride and sodium may be such as to reduce the initially formed charge in the final reduction zone to an average valence state of 2, for example (i. e., one mole titanium tetrachloride and 2 moles of sodium are fed to the final reduction zone). After the initial charge has been formed in the final reduction zone, the flow of titanium tetrachloride is stopped, and the feed rate of sodium is drastically reduced so that the reduction of the titanium from a valence state of 2 to a valence state of zero is achieved over a relatively long period (on the order of 3 hours or so).

Near the end of the final reduction period, the amount of sodium added to the final reduction zone is more than enough to completely reduce all of the residual titanium chlorides in the final reduction zone. During this last portion of the reduction period, agitation may be employed so as to assure that complete intermixing of the finally introduced excess sodium and any residual lower chloride of titanium is achieved. This assures the production of a molten slurry of titanium crystals in salt which is substantially completely free of lower chlorides of titanium.

The process, as described above, may take place as a batch operation in a single reactor or it may take place in a plurality of sequentially arranged reactors which provide stepwise reduction of the titanium chlorides in a plurality of separate reduction zones. Equally, the process can be practiced in a single, multi-stage reactor wherein the average valence state of the titanium is gradually reduced to zero. This multi-stage reactor can thus be a long tube into one end of which titanium tetrachloride is fed, the average valence state of the titanium content being gradually reduced as the titanium chlorides progress along the length of the tube.

Referring now to Fig. 1 there is schematically illustrated one preferred method of practicing the present invention. In this particular embodiment titanium tetrachloride is shown as the starting material, and sodium is illustrated as the reducing agent, these two materials being illustrated for simplicity of description only. Titanium tetrachloride and sodium are fed to a reactor 10 for producing a mixture of salt and titanium lower chlorides. The mole ratio of titanium tetrachloride to sodium is preferably about 1 to 2 so as to give a mixture of salt and titanium dichloride. If desired, an additional charge of salt may be provided in the reactor 10 so as to provide more salt than is produced by the initial reduction of the titanium tetrachloride. This initial reduction to the dichloride can take place at a relatively rapid rate and is preferably accomplished with agitation of the salt bath to provide uniformity of mixing of the reactants to produce a uniform dispersion of the dichloride in the salt.

Where the average valence of the titanium produced in the first stage reduction is 2 or above, this first stage reduction may take place as rapidly as the heat can be removed from the reactor. The mixture of salt and lower chlorides of titanium produced in the reactor 10 is fed to a final reduction zone 12 wherein the lower chlorides of titanium are gradually reduced to a valence of zero by slowly introducing two additional moles of sodium into the final reduction zone. This reduction preferably takes place over a time period in excess of an hour, preferably as long as 3 hours or more.

Complete reduction of the lower chloride is achieved in the final reduction zone. After the completion of the reduction, it is also preferred that some excess sodium be provided so as to assure complete freedom from lower chlorides of titanium.

The resultant slurry of titanium crystals, molten salt,

and excess sodium is then subjected to a separation step 14 which may be a simple decanting operation wherein the excess sodium is removed, as a liquid, from the mixture. Most of the excess by-product salt may also be drained off at this point, and a relatively concentrated mixture of titanium crystals and salt may then be transferred to an aqueous acid leaching bath, indicated at 16. It is obvious that the titanium crystals and the salt must be cooled prior to the aqueous acid leaching step. The resultant leached titanium crystals are then dried and preferably fed to an arc melting operation 18 where they can be formed into an ingot, casting, or the like. Additional alloying elements may be added to the titanium during the melting operation.

Numerous modifications in the above invention may be made without departing from the scope thereof. For example, the two reduction operations 10 and 12 can be carried out in a single batch reactor, if desired. Thus, 2 moles of sodium and 1 mole of titanium tetrachloride may be initially fed into the single reactor at a relatively high rate of speed. After a desired quantity of titanium dichloride has been so produced, the titanium tetrachloride feed may be stopped and the sodium supply may be reduced so that the reduction of the dichloride to titanium metal takes place over a time period on the order of several hours. With a properly constructed reactor the decanting and gross separation of the titanium crystals from the bulk of the salt may take place within the single reactor.

In order to describe more fully a number of alternative methods of practicing the invention, there are set forth below a few specific examples of experimental runs which have been made. These examples are nonlimiting and are merely illustrative of numerous additional embodiments of the invention. In these examples, the experiments were carried out in a nickel reactor having a diameter of 12 inches and a height of 27 inches. The reactor was equipped with a stirrer for agitating the salt bath in the reactor. Feed tubes were provided for feeding liquid titanium tetrachloride and liquid sodium (or liquid sodium-potassium alloy) to the reactor. Temperatures were indicated by thermocouples positioned within the salt charge. An atmosphere of argon was maintained in the reactor during the runs.

#### Example I

30 lbs. of NaCl were charged to the reactor which was then purged of air by the use of a vacuum and argon. The reactor was then heated to about 890° C. Titanium tetrachloride was fed to the reactor at a rate of 42.8 lbs. per hour along with sodium at a rate of 10.4 lbs. per hour. During this initial reduction of titanium tetrachloride (1 mole of  $TiCl_4$  and 2 moles of Na), the salt bath was agitated to provide a uniform dispersion of titanium dichloride in the molten salt, and the average temperature of the molten salt was about 910° C. After one hour the feed of titanium tetrachloride was stopped and the feed of sodium was reduced to 2.08 lbs. per hour. This modified feed rate was maintained for 5 hours, the average valence of the titanium dropping during this time from 2 to 0. During this portion of the run the sodium was fed to the top of the salt bath and no agitation was employed. During the final reduction portion of the reaction, the temperature of the salt bath was maintained at about 890° C. During the final reduction (i. e., after formation of the initial titanium dichloride charge), the average over-all titanium production rate was at 3.6 lbs. of titanium per cubic foot of final reduction mixture per hour.

Due to the exothermic nature of the reaction, even at the slow rate of reduction, it was possible (by radiation cooling) to maintain the reactor walls at a temperature slightly below the melting point (i. e., 800° C.) of the salt. The reactor walls were thus protected by a thin layer of frozen salt. At the termination of the run the total charge in the reactor was allowed to freeze and was cooled to

room temperature. Thereafter, the product was removed from the reactor and was subjected to leaching in 5% hydrochloric acid. After the acid leaching the product was leached in methanol and then ether and finally dried under a vacuum to remove all traces of water, alcohol, and ether.

The titanium crystals produced under the above conditions had a size distribution preponderantly greater than about 20 mesh. A number of the crystals had a length of 1 inch or longer, and an average thickness of  $\frac{1}{16}$  inch. 88% of the resultant titanium crystals were arc-melted in an inert atmosphere to form buttons. These buttons had a Rockwell A hardness of less than 52. Of the total product, 63% (+20 mesh) had a Rockwell A hardness of 37. The variation of the average titanium valence (on a cumulative basis) during this reduction reaction is plotted in Fig. 2.

#### Example II

5 lbs. of a mixture of sodium chloride and potassium chloride (68.5 mole percent NaCl, 31.5 mole percent KCl) were charged to the reactor which was then purged of air by the use of a vacuum and argon. The reactor was then heated to a temperature of about 850° C. and titanium tetrachloride was fed to the reactor at a rate of 11.2 lbs. per hour. Along with this titanium tetrachloride feed there was provided a feed of a sodium-potassium alloy at a rate of 5.28 lbs. per hour. This alloy consisted of about 56% sodium and 44% potassium (on a weight basis). The titanium tetrachloride feed was stopped at the end of 180 minutes and the sodium-potassium feed was continued for a total time of 226 minutes. During the total reduction time, the salt bath was agitated by use of a stirrer. As will be apparent from the above figures, the initial valence of the titanium formed was 1, this valence remaining at an average of 1 for the first 3 hours and then being slowly reduced to zero during the last 45 minutes. The product from this run was treated in a manner similar to that of Example I. A representative sample was then arc melted to give a button having a Rockwell A hardness of 48. The average titanium valence during this run is plotted in Fig. 2.

#### Example III

An empty reactor was purged of air and charged with argon and then heated to about 850° C. Titanium tetrachloride was fed to the reactor at a rate of 20.8 lbs. per hour for 14 minutes. During this feed of titanium tetrachloride a sodium-potassium alloy was fed at the rate of 3.2 lbs. per hour for 14 minutes. The sodium-potassium feed was then increased to 6.46 lbs. per hour and the titanium tetrachloride feed was decreased to 12.5 lbs. per hour. This relative rate was continued for about 104 minutes. Then the sodium-potassium feed was decreased to 4.81 lbs. per hour and the titanium tetrachloride feed was decreased to 9.67 lbs. per hour. This rate was continued for 82 minutes. The titanium tetrachloride feed was then stopped and the sodium-potassium feed was continued at a rate of 8.53 lbs. per hour for an additional 41 minutes. The run was held at temperature for an additional period of 120 minutes after cessation of the sodium-potassium feed. During this total run no agitation was employed and the temperature of the salt bath was maintained at about 850° C.

The product from this run was treated in a manner similar to that of Example I. A representative sample was then arc-melted to give a Rockwell A hardness of 37. The average titanium valence during this run is plotted in Fig. 2.

While specific experimental runs have been illustrated above, numerous alternative methods may be employed without departing from the spirit of the invention. The temperature of the reaction mass may be widely varied from slightly above the melting point of the salt to temperatures on the order of 1000° C. and above. How-

ever, there appears to be no particular advantage in operating at the higher temperatures and these higher temperatures give increasingly serious problems of materials of construction, heat transfer, etc. Numerous reducing agents, other than the sodium or sodium-potassium alloy, can be employed; for example, potassium, calcium, magnesium, lithium, and various combinations of these elements may be utilized. From the standpoint of cheapness, sodium, sodium-potassium alloy, or magnesium are preferred. Other halides of titanium may be utilized, although from the standpoint of cost, ease of handling, etc., the tetrachloride is most preferred.

Additionally, the reactor can be fed with lower halides of titanium such as titanium trichloride manufactured from titanium-bearing materials in the manner shown in the copending applications of Singleton, Serial No. 304,388, filed August 14, 1952, and Singleton, Serial No. 315,461, filed October 18, 1952. Equally, titanium trichloride can be made by the technique described by Sherfey et al., Journal of Research of the National Bureau of Standards, 46, 299-300, April 1951. Additionally, the dichloride of titanium can be manufactured by numerous processes such as disproportionation of the trichloride or partial reduction of the trichloride or tetrachloride.

The present invention can be equally employed for the manufacture of titanium alloys by the co-reduction of the chlorides, for example, of vanadium, chromium, manganese, iron, nickel, cobalt, columbium, tantalum, molybdenum, tungsten, or silicon. In this case the alloy may be a binary alloy or it may be an alloy containing 3 or 4 constituents. In the manufacture of alloys the same general conditions of the slow reduction of the titanium halide and reducible compounds of the alloying constituents must be employed.

When a continuous reactor is employed, as distinguished from the batch reactor, it is preferred to have numerous points of introduction of the reducing agent (e. g., sodium) so as to obtain as uniform as possible a distribution of the sodium into the reaction mixture. As pointed out above, it is highly undesirable to provide, in localized zones of the reaction mixture, any amount of reducing agent which is sufficient to rapidly reduce the titanium chlorides to metallic titanium. With the continuous reactor, it is preferred to have a slowly moving stream (which may be moving in a horizontal direction through a long tube). With such an arrangement of reactor, the reducing agent (e. g., sodium) is introduced at a great many points along the moving stream so that the moving stream is slowly and uniformly reduced from an average valence of less than 3 to a valence of zero in a time period of approximately 3 to 5 hours. Thus, if one mole of titanium tetrachloride is introduced at one end of the tube along with one mole of sodium (to form  $TiCl_3$ ) so that the titanium in the initially formed mixture has an average valence of 3, it will leave the other end of the long tube 3 to 5 hours later at a valence of zero.

In a continuous reactor it is preferred that the hot mixture of molten salt and titanium crystals be discharged onto a chilled surface so as to rapidly freeze the salt in a non-adherent form on the chilled surface, and to rapidly lower the temperature of the contained titanium to a point where it is not appreciably reactive.

It should be additionally pointed out that the salt mixture in which the slow reduction is carried out may be formed of numerous halides which can be mixed halides, single halides, and halides of materials other than the specific reducing agent or agents employed in the reaction. From the standpoint of simplicity of operation and ease of control, it is preferred, however, that the salt be the chloride of the reducing agent. Thus, while it is quite feasible to employ binary and ternary mixtures of halides having quite low melting points, not too much is gained and the additional expense is not particularly

warranted. This is particularly true in view of the excellent results which can be obtained by the use of sodium chloride as the salt for supporting the the slurry of titanium dichloride (in a preferred embodiment) which is slowly reduced to titanium metal.

It should be pointed out, in connection with a consideration of the various salts which can be employed, that these salts should be completely anhydrous and free of any contaminants such as carbon, nitrogen, oxygen, or hydrogen. This is due to the tremendous reactivity of titanium metal at temperatures on the order of 800° to 900° C. and above.

In connection with the formation of alloys, the co-reduction of alloying halides has been mentioned previously and the addition of alloying elements to the final titanium crystals in the melting step is shown in Fig. 1. Other alloying methods, such as the formation of master alloys and the like, may be equally employed during the reduction operation or during the subsequent melting operation. When the word "titanium" is used in the appended claims, it is intended to include alloys as well as the pure metal.

While the invention has been described in a preferred form wherein the average titanium valence is taken from a value of 2 or more to zero during the "final reduction" period, it can be modified by providing for less than complete reduction of the titanium chlorides in the "final reduction" period. Thus, for example, the reduction of a salt-titanium chloride mixture may be slowly reduced from an average valence of 2 to an average valence of about 0.5 over an extended period. Equally, the reduction may be achieved over an extended period at a constant average valence of about 1 (see Example II), without completing the reduction to a valence approaching or equalling zero. The resultant residual titanium chlorides in the mixture can then be reduced to titanium metal rapidly and in a separate zone. This method is less preferred, however, since rapid reduction of appreciable quantities of titanium chlorides inevitably produces an almost quantitative yields of titanium fines. Such fines are extremely difficult to separate, in a pure state, from the residual salt and unless separated from the larger titanium crystals will add sufficient impurities to the finally melted titanium so as to drastically reduce its value.

Equally, the titanium crystals can be separated from the mixture of titanium crystals, salt and lower chlorides and the crystal-free mixture, with its titanium chloride content, can be recycled to the reactor. This method is also less preferred since it is extremely difficult to separate the titanium crystals from the mixture of salt and lower chlorides without contaminating the titanium crystals, oxidizing the lower titanium chlorides, or producing large quantities of titanium fines.

Since certain changes may be made in the above process without departing from the scope of the invention herein involved, it is intended that all matter contained in the above description, or shown in the accompanying drawings, shall be interpreted as illustrative and not in a limiting sense.

What is claimed is:

1. The process of producing crystalline titanium which comprises the steps of providing a mixture of a molten salt and at least one lower halide of titanium in an air-free reduction zone, said mixture being substantially free of titanium fines, maintaining the salt in the reduction zone at a temperature above its melting point, introducing a reducing agent into the reduction zone at a relatively slow rate so that the average valence state of the titanium in the reduction zone is gradually reduced, said reducing agent comprising at least one metal selected from the group consisting of the alkali metals and the alkaline earth metals, the introduction of the reducing agent into the reduction zone being sufficiently gradual to require a reduction period of at least two hours for

reducing the average titanium valence from a value of less than 3 to a value of zero, said reducing agent being substantially uniformly introduced into the mixture to eliminate high concentrations of undissolved reducing agent capable of achieving rapid reduction of the average titanium valence in localized portions of the molten salt in the reaction zone, and separating the titanium crystals from the salt.

2. The process of claim 1 wherein the reducing agent comprises sodium and the salt comprises sodium chloride.

3. The process of claim 1 wherein the mixture of salt and lower halides of titanium is advanced slowly through the reduction zone, the gradual reduction of the average titanium valence in the advancing mixture being achieved by introduction of the reducing agent at spaced points along the path of travel of the mixture.

4. The process of claim 1 wherein the mixture of salt and lower halides of titanium is formed in the reduction zone by initially introducing titanium tetrachloride and an amount of reducing agent less than that required for complete reduction of the introduced titanium tetrachloride, the relative rates of introduction of the tetrachloride and the reducing agent being shifted to achieve the gradual reduction of the average titanium valence to zero.

5. The process of claim 1 wherein the salt comprises a halide of one of the metals from the group consisting of the alkali metals and the alkaline earth metals.

6. The process of claim 1 wherein the salt is a chloride of the reducing agent.

7. The process of claim 1 wherein the uniform introduction of the reducing agent into the salt is obtained by dissolving the reducing agent in the salt.

8. The process of claim 1 wherein a halide of an alloying metal is slowly reduced along with the halide of titanium to provide crystals of titanium containing said alloying metal.

9. The process of claim 1 wherein the halide of titanium comprises a lower chloride of titanium and a chlo-

ride of titanium is introduced into the reduction zone during the reduction of the lower titanium chloride.

10. In a process for producing titanium wherein a lower halide of titanium is dissolved in a fused salt bath which is substantially free of titanium fines and the titanium halide is slowly reduced to titanium crystals over an extended period of at least one hour by means of a metallic reducing agent, the average titanium valence decreasing from a value of between two and three to a value approaching zero during the reduction period, the metallic reducing agent comprising at least one metal selected from the group consisting of the alkali metals and the alkaline earth metals, the improvement which comprises adding molten reducing agent to the surface of the fused salt bath over an extended period of time while said bath remains quiescent.

11. The process of claim 10 wherein the halide of titanium comprises titanium dichloride dissolved in a fused sodium chloride bath and the reducing agent comprises sodium.

#### References Cited in the file of this patent

#### UNITED STATES PATENTS

|           |                |               |
|-----------|----------------|---------------|
| 2,148,345 | Freudenberg    | Feb. 21, 1939 |
| 2,443,253 | Kroll et al.   | June 15, 1948 |
| 2,564,337 | Maddex         | Aug. 14, 1951 |
| 2,607,674 | Winter         | Aug. 19, 1952 |
| 2,618,549 | Glasser et al. | Nov. 18, 1952 |
| 2,618,550 | Hampel et al.  | Nov. 18, 1952 |
| 2,647,826 | Jordan         | Aug. 4, 1953  |
| 2,667,413 | Jordan         | Jan. 26, 1954 |
| 2,668,750 | Krchma         | Feb. 9, 1954  |

#### OTHER REFERENCES

- Zeitschrift für Anorganische und Allgemeine Chemie, vol. 234, 1937, pages 42-50. Page 44 pertinent.  
 Report of Investigations 4519, "Production of Ductile Titanium at Boulder City, Nev." Published August 1949 by Bureau of Mines, Washington, D. C. Pages 9-14 pertinent. Entire report 39 pages.  
 Journal of Metals, April 1950, pages 634-640.